

Aug. 12, 1941.

C. ADAMOLI

2,251,968

PROCESS FOR THE PRODUCTION OF VERY PURE MAGNESIUM FROM MAGNESIUM ORES

Filed Sept. 7, 1938



Patented Aug. 12, 1941

2,251,968

# UNITED STATES PATENT OFFICE

2,251,968

## PROCESS FOR THE PRODUCTION OF VERY PURE MAGNESIUM FROM MAGNESIUM ORES

Carlo Adamoli, Milan, Italy, assignor to Perosa  
Corporation, Wilmington, Del., a corporation of  
Delaware

Application September 7, 1938, Serial No. 228,865  
In Italy September 11, 1937

23 Claims. (Cl. 75—67)

After some early experiments based on reduction by carbon at high temperatures, work on the commercial preparation of metallic magnesium has been carried out almost exclusively in the direction of electrolytic decomposition of fused magnesium chloride. The technical difficulties are known which must be overcome in such an electrolysis; the chemical and physical difficulties are also known which are met with in obtaining a magnesium chloride which is pure enough to give a metal which is not contaminated by other elements which cannot be removed by further melting operations, and which is sufficiently anhydrous not to give rise to magnesium oxychloride when heated. In spite of all the contrivances which have been introduced into these operations, it is well known that magnesium cannot be freed from all the impurities which has always been sufficient to impede a use which, without these impurities, could take place on a large scale owing to the exceptionally good mechanical characteristics which the pure metal possesses. It is well known that less than 0.2% of impurities altogether is sufficient, even when mainly due to iron, aluminum, silicon and chlorine, to cause the elasticity to drop to 70% of the value which corresponds to the pure metal, and to cause the metal to show the chemical instability due to which the products made of ordinary magnesium are rapidly altered and worn. For this reason it has been attempted to obtain a pure metal by distilling and subliming it, but when working according to such methods the losses due to the metal which has been consumed in the course of the further melting operations and granular condensations are so great that the cost of a pure magnesium obtained first by the electrolysis of the anhydrous chloride (under the best conditions) and then by distillation or sublimation in a vacuum is so high that it prevents the use of magnesium so obtained in large mechanical constructions.

The process according to the present invention differs from the above mentioned processes by the fact that electrolysis is not used and that the starting materials are not purified magnesium salts, but ores which are very common in nature, such as magnesite, gibertite, talc, dolomite; that the magnesium which is obtained is free from any impurity having its origin either in the ores or in the reagents which have been used, the process being performed in the course of a single direct operation and avoiding the losses of metal which are ordinarily incurred when it is necessary to melt the metal because it is not compact enough. Finally, the process according to the invention still differs from the other processes by the fact that only a single reagent is used, which is decomposed and regenerated, and that thermal energy is consumed only in amounts correspond-

ing to the heat necessary for liberating and evaporating the metallic magnesium which is produced.

Heretofore it has not been customary to use magnesium fluoride as the material from which to produce metallic magnesium. This is due to the fact that the fluoride of magnesium is practically never to be found in nature in the condition of a massive ore, and that its cost, when artificially produced—is always too high; on the other hand, its high melting point (1260° C.) results in its use not being advantageous for the production of metallic magnesium by electrolysis of the molten magnesium fluoride which, furthermore, possesses only a small electric conductivity. However, when using a distillation process for the production of magnesium, in order to obtain pure metal, the fact that fluorine can readily combine with other elements which have a chemical affinity for it higher than the affinity of magnesium for fluorine, has suggested to the applicant the concept that the use of magnesium fluoride, if it were possible to produce it at a low cost, would be highly advantageous for a reduction process as compared with the use of magnesium oxide the reduction of which, either by carbon or by any other reagent (with the exception of alkali metals which are expensive) takes place at exceedingly high temperatures at which the pressure of the magnesium vapor, the boiling point of which is about 1160° C., is so high that it is difficult to condense it, while it is oxidized readily; on the other hand the problem of the resistance to wear of the construction materials used for the commercial contrivances which are suitable for this process, becomes thus insoluble.

In the case of silicon great difficulties are also met with because of the formation of oxidized silicon compounds with metallic oxides, the said compounds consuming uselessly a portion of the reducing metal and of the reduced metal, so that no chemical equivalency between the consumed silicon and the produced magnesium can be obtained.

The present invention relates to a process for the commercial production of metallic magnesium from magnesium ores by converting the said ores into magnesium fluoride by means of fluorine introduced once for all into an operating cycle in the form of magnesium fluoride, which is decomposed by the exchange of its fluorine thus producing vaporized magnesium in a pure condition, which is condensed, and a fluoride of a reducing agent, from which fluorine the fluorine is extracted by any known process and caused to react on a further quantity of magnesium ore in order to form magnesium fluoride which is submitted anew to an exchange reaction with the reducing agent above referred to and so on, the fluorine thus serving in a closed cycle

for converting the magnesium of the ore into magnesium fluoride and then for liberating magnesium by the action of the reducing agent and finally for the formation of a fluorine compound which converts anew through its fluorine a further quantity of magnesium from a further quantity of ore, and so on.

The production of magnesium which has been distilled from its fluoride supposes a reaction of the following kind:



where  $m$  is a monovalent metal. In order that it may be carried into effect in a commercial manner and under the conditions which have been provided heretofore, this reaction would require the use of an alkali or alkaline earth metal such as sodium, potassium or calcium, the cost of production of which would be high according to the amount chemically equivalent to the magnesium which is to be liberated.

According to the process which forms the subject matter of this invention, the starting material is, therefore, a magnesiferous ore. Natural magnesite, natural carbonate of magnesium called gibertite and dolomite are well suited for this purpose; however, the fundamental operating cycle allows of the use of a material other than a magnesiferous material which is equivalent from the point of view of the process, such as, for instance, talc, steatite or other materials of the same kind. The chemical principles on which the process is based are as follows: (1) The conveying of the fluorine of the fluoride of magnesium into another compound which is such that it renders possible the displacement of the chemically equivalent quantity of fluorine, for instance in the form of hydrofluoric acid adapted for producing further magnesium fluoride; (2) The use as reducing agent of a tetravalent metalloid such as, for instance, carbon or silicon, alone or mixed with other metalloids or metals or present in compounds or combinations of the metallic type, such as carbides and silicid compounds or as alloys.

The accompanying drawing diagrammatically shows in a conventional manner a qualitative balance-sheet of the cyclic process according to the invention. Magnesiferous ore enters in the cycle at  $a$ ; it then meets at  $b$  the fluorine of the cycle, e. g. in the form of hydrofluoric acid coming from  $c$ , to which is added a small amount of supplemental hydrofluoric acid introduced in the cycle at  $d$  to compensate for losses of fluorine. The magnesium fluoride thus formed at  $b$ , which eventually is separated from a residue which does not substantially contain fluorine and which is removed from the cycle through  $e$ , passes through  $f$  in order to be submitted to the action of a reducing agent entering the cycle at  $g$ . The reaction produced at  $h$  between the magnesium fluoride and the reducing agent delivers on the one hand, vapors of pure magnesium which leave the cycle through  $i$  and pass to the condenser and on the other hand, a fluorinated mixture which passes through  $j$ , meets at  $k$  the reagent which enters the cycle at  $l$  and liberates the fluorine of the mixture and combines with it to form hydrofluoric acid. The thus recovered fluorine is separated from a residue which contains substantially no fluorine and which is removed through  $m$ ; the said fluorine to which is added the small amount of supplemental hydrofluoric acid entering the cycle through  $d$ , passes through  $c$  and at  $b$  meets a further portion of magne-

siferous ore which is introduced into the cycle at  $a$ , in order to form further magnesium fluoride and so on.

- In the case of a mixture of metallic and metalloids reducing agents, there are two parallel reactions, one with the metallic reducing agent and the other with the metalloids reducing agent, while either the use of the resulting metallic fluoride or metalloids tetrafluoride are resorted to, 5 as desired, for the regeneration of the fluorine. By causing magnesium fluoride to react alone or mixed with other fluorides or oxides (such as oxides of the magnesium itself or with calcium 10 which is contained in dolomite, for instance) on calcium or on calcium silicide, calcium carbide or another silicide or carbide, or on alloys of both metalloids with other elements, the following 15 products are obtained: metallic magnesium which distills, calcium fluoride and a metalloids tetrafluoride; out of the calcium fluoride and through the known reaction by means of strong acids, or out of the metalloids tetrafluoride by treating the same by means of water vapour according to the 20 process as described in the Italian Patent No. 355,502, dated September 10, 1937, the hydrofluoric acid is regenerated and is used to form again magnesium fluoride from the ore of the kind which has been used as raw material.
- 25 The decomposition of the magnesium fluoride by means of metallic calcium takes place giving a practically total output according to the reaction:



- 30 if care is taken in adding a fluoride such as, for instance, an alkali metal fluoride adapted to maintain the melting temperature of the mass at a sufficiently low degree of temperature during the whole decomposition. For instance, for this 35 purpose, an addition of sodium fluoride can be made which allows the reducing metal to react on the magnesium fluoride at a temperature which is sufficiently low to prevent any gradual distillation of the molten calcium which is added as the 40 operation progresses. The final product which 45 is obtained after the distillation of the magnesium is calcium fluoride with small quantities of other fluorides such as sodium fluoride and from this product the fluorinating reactions are repeated 50 in a continuous cycle by the process which has been described above in the case of the use of calcium carbide.

- The decomposition of the magnesium fluoride by means of calcium carbide is one example of 55 the step of displacement of the fluorine of magnesium fluoride. In an iron retort of a suitable type contained in a muffle which is heated with coal, oil or electricity, carbide of calcium, as available in the market is introduced preferably after having been comminuted to a fine granular condition like sand, and intimately mixed with a chemically equivalent proportion of magnesium fluoride, or preferably with a proportionally larger quantity of magnesium and calcium fluoride, when the hydrofluoric reaction is carried out on dolomite which, as is known, is a natural carbonate of calcium and magnesium. This magnesium fluoride is, for instance, obtained in a stage which will be described later on. A violent reaction takes place at the melting temperature of the magnesium and it is accompanied by a development of heat by which the calcium carbide and the magnesium fluoride are decomposed while causing the formation of magnesium 60 which distills, and of calcium fluoride which re-
- 65
- 70
- 75

mains in a molten condition and is found to be mixed with the graphitic carbon which has been produced. When only magnesium fluoride is present the reaction can be briefly represented by the following equation:



When both calcium and magnesium fluorides are present, the calcium fluoride is an inert ingredient. The magnesium vapors which distill are led to a condenser which can be formed of a suitably cooled iron vessel in which a rain of molten magnesium, at 700° C. precipitates from the magnesium vapors and the liquid magnesium which has been formed is poured into a mould with the usual precautions well known in the art. At the beginning of charging the material and during the treatment, the retort and the condenser are maintained full of inert gases such as, for instance, methane, in order to avoid any oxidation of the escaping metal. When the larger part of the magnesium of the retort has been distilled off, which is the case after a time which varies according to the amount of the mass, but which is always short, a good deal of the calcium fluoride and of the carbon is removed from the bottom of the retort and caused to flow as such into cold water. The calcium fluoride which has been chilled in this manner can be readily pulverized. It can then be introduced into a mixer and transformed into a paste by being thoroughly mixed with sulphuric acid and then submitted to a temperature of 150–170° C. until all the fluorine has been removed in the form of gaseous hydrofluoric acid in a dry condition, which is caused to react in another room, for instance in a tower which is inwardly protected by compact burnt magnesite, with a finely powdered magnesiferous ore, preferably a powder of a natural carbonate of Mg or powdered dolomite, which is sprayed out into the room or tower by means of an atomizer together with carbon dioxide. The tower can be heated by the hot gases coming from the furnace heating the retort for the distillation of the magnesium; with this heat and with the heat which is produced by the following exothermic reaction, which corresponds to the use of the natural carbonate of magnesium:



the fluorination reaction takes place and the magnesium fluoride as well as the other fluorides which may have been formed, precipitate on the bottom of the tower, wherefrom they are removed and then mixed with the reducing agent, for instance calcium carbide, in the manner which has already been hereabove described. The reaction takes place in the same manner when operating on dolomite or another magnesiferous ore of the same kind. In the cycle of treatment a chemical equivalent of each of the chemical materials which are used for the reaction is consumed, these materials being calcium carbide and sulphuric acid, when starting from natural carbonate of magnesium. In case dolomite is used, the consumption of sulphuric acid is higher due to the presence of calcium carbonate in the dolomite, which calcium carbonate is converted into calcium fluoride in the fluorination of the magnesium carbonate. From the hydrofluoric reaction room (b. of Fig. 1) carbon dioxide is removed, which is in excess with respect to the proportion of carbon dioxide which is necessary for accompanying the magnesium carbonate or the dolomite into said room.

As to the decomposition of the magnesium fluoride by free or elemental silicon alone, this reducing agent is used commercially according to the invention, on the basis of the fact that the silicon in a finely powdered condition and mixed with magnesium fluoride and with quick lime in a proportion which is chemically equivalent, causes the distillation of the metallic magnesium at the melting temperature of the magnesium fluoride the reaction being as follows:



The pasty mass which remains after the magnesium has been removed by distillation is formed of a mixture of silica and calcium fluoride, from which mixture all the fluorine which is necessary for the fluorination of further quantities of gibertite or other magnesiferous ore is obtained by the above described process.

The production of hydrofluoric acid by means of the fluorine which circulates in a closed cycle in the process is based on the reaction of the sulphuric acid on the mixture which forms the residue of the preceding reaction; in fact, through its reaction on the residue which is obtained after the distillation of the magnesium, the sulphuric acid produces silicon tetrafluoride which regenerates the corresponding hydrofluoric acid, for instance by the use of the process according to the Italian Patent No. 355,502.

The reduction of the magnesium fluoride by means of silicon, as well as the condensation of the magnesium, are performed in the same manner as in the first case which has been described for the treatment of extraction by means of carbide of calcium. An apparatus for carrying out the operations is shown diagrammatically in Figure 2 of the appended drawing. The intimate mixture of silicon, magnesium fluoride and quick lime is agglomerated, for instance, by pressure and is introduced e. g. into a suitable cast iron retort, 1 provided with an inner protective lining 2 of compressed and fritted steatite. The retort is provided, on the one hand, with a conduit 3 for the outlet of the vapors of magnesium and, on the other hand, with an outlet 4 for the fluid slag. The charging of the agglomerated product pieces on the molten mass is effected automatically, for instance, by means of a belt

5, which takes the agglomerated product pieces and discharges them onto the molten mass. The charging chamber 6 for the agglomerated products which takes the briquettes outwardly and brings them to the molten bath of  $\text{MgF}_2$ , is preferably arranged for this purpose, in the form of successive semi-closed sections by means of partition walls 6a which come almost in engagement with the free faces of the belt 5 and of the material which is conveyed by the said belt; the sections which are formed in this manner are fed with a neutral gas, such as methane, at a pressure which is not lower than the atmospheric pressure at this moment, in order that it may be possible gradually to remove all the air at least from the last section, before the agglomerated pieces are discharged onto the molten mass, the air escaping through the narrow free intervals left between the wall partitions of the sections and the feeding belt or the material in course of feeding. Thus the whole operation is performed in an inert atmosphere and at atmospheric pressure or at a neighboring and slightly higher pressure.

The decomposition of the magnesium fluoride by means of chemically free silicon alone is

greatly accelerated when the operation is so carried out that there are present, in the beginning, bases such as lime or magnesium oxide in proportions which are always lower than the proportions which correspond to the chemical equivalence of the amount of the silicon which is present, while the magnesium fluoride is then gradually introduced after having been mixed with the silicon, while maintaining between them the proportions which represent the chemical equivalency. By using a magnesium fluoride containing oxide of magnesium it is possible to moderate the intensity of the reaction, which can be explained by the formation, instead of silica, of silicon oxyfluoride; this body itself can react on the alkaline earth metal fluorides under the conditions of temperature at which the operation is carried out, and by a secondary reaction with the magnesium fluoride, it passes to the condition of a tetrafluoride, thus regenerating the oxide of magnesium. In fact, the reaction takes place in two stages: in the first stage the magnesium is freed from the fluoride and from the oxide which is present and then, by a further addition of magnesium fluoride, if the latter has not already been present in excess, tetrafluoride of silicon is liberated and the magnesium oxide which was present at the beginning re-composes itself. This is produced according to the equations:



On the basis of these equations, it is shown that the phase of formation of the metallic magnesium is separated from the phase of formation of tetrafluoride of silicon, the recoverable metallic magnesium being completely liberated before the tetrafluoride of silicon can be formed. These analytical interpretations are given, of course, for the purpose of explanation; others could also be given; it is a fact, however, that the application of this process for the commercial production allows of directly obtaining practically all the metallic magnesium which is contained in the molten mass, as well as of obtaining, also directly, the silicon fluoride without it being necessary to pass through an intermediate reaction of the sulphuric acid on a silicate and fluoride slag, as explained above for the case where the decomposition of the magnesium fluoride is effected by free silicon alone. In this case the process and the apparatus for the production hereabove mentioned are modified as regards construction and working of the retort in that at the beginning of the production the briquettes are formed of silicon, magnesium fluoride and magnesium oxide and that in the further operation they are formed of magnesium fluoride and silicon without oxide; the first briquettes are charged in a single operation at the beginning and the other briquettes are charged successively at intervals, while the conduits through which the magnesium escapes in a gaseous condition are first opened in order to let the magnesium vapors go to the condensing appliance after which they are closed and the conduits are opened through which the silicon tetrafluoride escapes in order to go to the appliances for the transformation thereof into hydrofluoric acid. Thus the reaction masses are maintained at a constant level and the slag which has been formed is removed in a continuous manner or intermittently. Briefly stated, the operation takes place as if it were effected in a single phase according to

the following reaction formula, which is synthetically expressed:



5 Of course, in this operation for the production of magnesium, variations of temperature and of duration as to the successive phases are alternately met. Thus a cycle of circulation of the fluorine according to a commercial production is obtained and silicon is consumed only in an amount which is chemically equivalent with respect to the magnesium which is produced.

15 The decomposition of the magnesium fluoride by means of calcium silicid represents the mixed type of operation according to this process by giving rise to a different circulation of the fluoride in the cycle of treatment. The reaction takes place which corresponds to the double exchange between the metallic elements by using a common silicid such as, for instance, calcium silicid which can be produced in large quantities from silica and calcium in an electric furnace at costs which are very suitable for the purpose and on such a basis that its composition is as follows: about 25 to 30% of calcium, 25 to 70% of silicon, 5 to 10% of iron, these contents corresponding approximately, as regards the relation silicon-calcium, to the formula  $\text{Si}_3\text{Ca}$ . When leaving the secondary reactions out of consideration one has first a transformation according to the following equation:



35 The light metallic magnesium silicid can be separated and gives magnesium by distillation, while the silicon, as a metallic residue, is recovered in an iron-silicon alloy having still a large silicon content, which can be used directly in metallurgy. It has been found, however, that it is preferable in many cases to re-use the magnesium silicid itself, preferably at the moment of its formation as a transforming agent for a further quantity of magnesium fluoride, no longer through the double exchange reaction between metals, but through the reaction of formation of silicon tetrafluoride. In this case the reaction which represents the transformations during the different phases is represented by the following equation:



50 By this process the fluoride which is necessary, is obtained partly according to the operative process which has been described in the case of the use of carbide and for the most part (6/7) by the operative process which has been hereabove described in the case of the use of metallic silicon alone.

60 The production of metallic magnesium on the basis of the above described process and according to one or the other of its practical applications can be usefully effected also by the use and the conversion of iron and silicon alloys. It has been found that iron and silicon alloys having a high silicon content can react with the magnesium fluoride in the same manner as the silicon itself, and also like the silicon which is contained in the calcium silicid, that is to say practically through the totality of their silicon contents.

65 Between a common silicon and iron alloy containing 60% of Si and 40% of Fe (60/40 alloy) and an also common alloy of iron and silicon containing 80% of Fe and 20% of Si (80/20 alloy), a quantity of silicon is available the reactivity

of which can be readily used for the above described process of production of magnesium by the action of its fluoride; by causing the silicon and iron alloy having a high content of silicon to react with the above described mixture of magnesium fluoride and base in a proportion corresponding to that which is necessary for simultaneously obtaining the magnesium and an iron and silicon alloy having a high content of iron, there is from the commercial point of view, the great advantage that the reaction can be carried out at low temperatures and from the economical point of view the advantage that a metallic by-product is obtained which can be readily sold or used; it is thus advantageous to use, instead of silicon, silicon which is contaminated with iron and the price of which is much lower than that of pure silicon. The reaction, chemically expressed according to the equivalencies and according to the above mentioned reaction (R) appears as follows:



As above mentioned, the process according to the present invention allows of directly using magnesium ores and it is characterized amongst other features in that the magnesium is always produced in a quantity which is equivalent to the fluorine which is present at the beginning and combined with the magnesium and finally in that neither the silicon nor the carbon practically react by reduction on the oxide, but by a double exchange with the fluorine.

One of the remarkable properties of the process according to the invention is that it is carried out at a temperature which is not higher than 1260° C., so that it has marked advantages with respect to the former processes.

In the same way iron and silicon alloys containing a reducing metal, such as, for instance, an alloy of iron, silicon and aluminum can be used for binding the fluorine of the magnesium fluoride and if desired of another metal which is combined with fluorine, and for liberating the magnesium. Thus, for instance, 12 tons of  $\text{MgF}_2$  (produced by causing 6 tons of gibertite to react on the fluorine which has been regenerated in the form of hydrofluoric acid) are treated by means of 4 tons of an alloy of 50% of Si, 35% of Al and 15% of Fe. The reaction will give 4.5 tons of Mg which will distill, and a residue of an alloy of 60% of Fe and 40% of Si and of a fluorinated mixture containing the fluorine of the magnesium fluoride, from which mixture the fluorine will be removed in the form of HF which will be used for reacting on a further mass of 16 tons of gibertite, adding a small proportion of HF for compensating the losses of fluorine which have possibly taken place in the course of the operations.

In the course of experiments for the commercial application of the fundamental means of the above described cyclic process for the production of magnesium, and the modifications, of the said process, the applicant has found that the said process is equally well suited for the manufacture of products formed of pure magnesium alloyed with other metals by still using the magnesium fluoride and submitting it to the same physico-chemical conversion processes as above described.

In fact, it has been possible to obtain other metals such as Li, Ce, Zr, Cd, Pb in the same manner as magnesium and simultaneously with

the latter, by the conversion of their compounds with fluorine by means of tetravalent metalloids or of their combinations or alloys with other metalloids, or metals, for instance carbides or silicides. It has thus been possible to obtain binary alloys and also alloys of a higher order having magnesium as their basis with very different relations between the constituents.

The raw material for alloying one or more metals with magnesium can be, for instance, an ore such as blende in the case of zinc, or in a general manner a fluorinated product obtained simultaneously or together with the magnesium fluoride (under the conditions which are indicated above for magnesium) or obtained in a similar manner or added in the course of the cyclic process according to the present invention. The production of various alloys of magnesium such as, for instance, Mg-Al, Mg-Sn, by the condensation of magnesium (produced according to the fundamental process as above described) in another metal in a liquid condition or in the body of alloys and more particularly alloys having a low melting point and maintained in a liquid condition in a similar manner, has also been tested with favorable results. This condensation takes place in the manner already described for the condensation of the vapours of magnesium.

Among the binary combinations which can be used the following combinations may be cited, which are quoted with the relative temperatures at which the said combinations, under given proportions, are in liquid condition and miscible with magnesium between defined limits:

Ag Al 560°; Ag Cd 630°; Ag Cu 780°; Ag Sb 490°; Ag Sn 480°; Al Be 650°; Al Cu 550°; Al Sn 450°; Al Zn 450°; Cu Be 865°; Cd Sb 500°; Cd Sn 180°; Cd Zn 265°; Cu Sb 650°; Cu Sn 675°; Cu Zn 595°; Fe Zn 765°; Li Sn 685°; Li Zn 520°; Sb Sn 425°; Sb Zn 565°; Sn Zn 200°.

Finally, it is still possible to produce magnesium from its fluoride in the already above described conditions by causing it to be retained by other metals as well as by suitable stable alloys brought to a molten condition, in the presence of magnesium fluoride before or during the phase of reaction for the decomposition of the magnesium fluoride. The term "suitable stable alloys" is here intended for designating alloys adapted to alloy with magnesium and which are not transformed into fluorides under the conditions of the operation.

In all the cases which have been described hereinabove, magnesium and its alloys are still obtained by using the process which has been described hereinabove for the production of magnesium which is not alloyed with other metals, or still better by using a process which forms an extension of the latter inasmuch as the alloy is obtained during the operation for the production of magnesium and not by a subsequent operation in which magnesium having already been separately obtained in any other manner is alloyed with another metal. By adding a zinc ore, for instance, to the magnesiferous ore which is the raw material, the transformation will take place in a similar manner to and simultaneously with that of the magnesium, and in the final condensation of the metal an alloy of magnesium and zinc will be obtained in the same proportion as that in which these elements are present in the initial ore mixture.

In another case the addition may take place in a subsequent phase after the fluorination of

the magnesium ore, by introducing in the cycle a fluoride which is stable but which is reducible under the conditions of the operation, such as cadmium fluoride ( $CdF_2$ ) obtained from cadmium ore; in this case the transformation will take place according to the same rule, but, of course, one will also obtain in the cyclic recovery of the fluorine the fluorine from the cadmium fluoride, which fluorine will be used for fluorinating a further quantity of cadmium ore. In the above mentioned case finally an alloy of magnesium and cadmium is finally obtained. In a similar manner alloys of magnesium with lithium, zinc or other metals having a similar behavior, are produced. In this manner binary alloys or alloys of a higher order can be obtained in which in all cases, the metal to be alloyed is distillable together with the magnesium.

But it is also possible, in order to obtain an alloy with pure magnesium, to make the addition of another metal which has already been extracted in part, by introducing it into the phase of condensation of the magnesium vapors, as is the case, for instance, of alloying aluminum with magnesium; in doing so the aluminum has an advantageous action as it plays the role of condensing agent at a temperature which is by 200° C. lower than the temperature of condensation when magnesium alone is present.

In this case, aluminum can also be replaced by one of its suitable alloys; a multiple magnesium alloy e. g. an alloy  $Mg-Al-Cu$  thus is obtained. Such magnesium alloys can be furthermore produced by the process which has been described for the production of magnesium which is not alloyed with other metals, even before the phase of distillation, as in the case hereinabove described for the alloys of magnesium and silicon; the latter can be produced directly in the liquid condition and may contain other metals besides and instead of silicon, no matter whether these metals are introduced as ores with the magnesium ore or as fluorinated compounds or as free metals. For instance, in the case of the reaction which has been hereinabove mentioned for the production of magnesium alone by treating magnesium fluoride with calcium silicide, the magnesium silicide can be produced intentionally and obtained as final product rather than in the form of an intermediary compound. Of course, the alloy of magnesium and silicon can also contain other metals when the latter have been introduced with the silicon or with the silicon compounds which are used in the transformation cycle.

What I claim is:

1. A cyclic process for obtaining very pure magnesium which comprises treating magnesiferous ore with hydrofluoric acid to form magnesium fluoride, treating said magnesium fluoride with calcium at the temperature of distillation of the magnesium and in a non-oxidizing atmosphere, condensing the magnesium vapors resulting from the reducing treatment, treating the calcium fluoride remaining after the distillation of the magnesium with a strong acid to regenerate the hydrofluoric acid, treating a further quantity of magnesiferous ore with said hydrofluoric acid to form magnesium fluoride, and treating said magnesium fluoride with calcium at a temperature of the distillation of the magnesium and in a non-oxidizing atmosphere.

2. A cyclic process for obtaining very pure magnesium according to claim 1, in which calcium fluoride is mixed with the magnesium fluoride submitted to reduction.

3. A cyclic process for obtaining very pure magnesium which comprises treating magnesiferous ore with hydrofluoric acid to form magnesium fluoride, treating said magnesium fluoride with silicon at the temperature of distillation of the magnesium and in a nonoxidizing atmosphere, condensing the magnesium vapors resulting from the reducing treatment, treating the silicon tetrafluoride remaining after the distillation of the magnesium to regenerate the hydrofluoric acid, treating a further quantity of magnesiferous ore with said hydrofluoric acid to form magnesium fluoride, and treating said magnesium fluoride with silicon at the temperature of the distillation of the magnesium and in a non-oxidizing atmosphere.

4. A cyclic process for obtaining very pure magnesium which comprises treating magnesiferous ore with hydrofluoric acid to form magnesium fluoride, treating said magnesium fluoride with an alloy of calcium with a metalloid of the group consisting of carbon and silicon at the temperature of distillation of the magnesium and in a non-oxidizing atmosphere, condensing the magnesium vapors resulting from the reducing treatment, treating the fluorinated product remaining after the distillation of the magnesium to regenerate the hydrofluoric acid, treating a further quantity of magnesiferous ore with said hydrofluoric acid to form magnesium fluoride, and treating said magnesium fluoride with an alloy of calcium with a metalloid of the group consisting of carbon and silicon at the temperature of the distillation of the magnesium and in a non-oxidizing atmosphere.

5. A cyclic process for obtaining very pure magnesium according to claim 4, in which an alloy of silicon and calcium is used for the reduction of the magnesium fluoride.

6. A cyclic process for obtaining very pure magnesium according to claim 4, in which an alloy of silicon and calcium is used for the reduction of the magnesium fluoride, the proportions of silicon and calcium, respectively, being chemically equivalent to the amounts of magnesium and fluorine of the magnesium fluoride.

7. A cyclic process for obtaining very pure magnesium according to claim 4, in which an alloy of silicon and calcium is used for the reduction of the magnesium fluoride, the total of the silicon and of the calcium of the said alloy being so proportioned with respect to the magnesium of the magnesium fluoride that they are chemically equivalent to each other.

8. A cyclic process for obtaining very pure magnesium, which comprises treating magnesiferous ore with hydrofluoric acid to form magnesium fluoride, treating said magnesium fluoride with a reducing agent of the group consisting of calcium and the metalloids of the group consisting of carbon and silicon at the temperature of distillation of the magnesium and in a non-oxidizing atmosphere, condensing the magnesium vapors resulting from the reducing treatment, treating the fluorinated product remaining after the distillation of the magnesium to regenerate the hydrofluoric acid, treating a further quantity of magnesiferous ore with said hydrofluoric acid to form magnesium fluoride, and treating said magnesium fluoride with a reducing agent of the group consisting of calcium and the metalloids of the group consisting of carbon and silicon.

9. A cyclic process for obtaining very pure magnesium according to claim 8, in which the treatment of the fluoride by the reducing agent

is carried out at a temperature between the melting temperature of the magnesium fluoride and 1260° C.

10. A cyclic process for obtaining very pure magnesium according to claim 8, in which alkali-metal fluoride is added to the magnesium fluoride in order to lower the temperature of the reaction.

11. A cyclic process for obtaining very pure magnesium according to claim 8, in which a supply of hydrofluoric acid is added to the fluorinated reagent which is used in the operative cycle, in order to compensate for the losses of fluorine.

12. A cyclic process for obtaining very pure magnesium according to claim 8, in which, to directly obtain magnesium alloyed with other metals, ores of the metals to be alloyed with the magnesium are mixed with the magnesium ore introduced into the operative cycle.

13. A cyclic process for obtaining very pure magnesium according to claim 8, in which, to directly obtain magnesium alloyed with other metals, fluorinated compounds of the metals to be alloyed with the magnesium are introduced into the operative cycle with the magnesium fluoride in the phase in which the latter is formed.

14. A cyclic process for obtaining very pure magnesium according to claim 8, in which, to directly obtain magnesium alloyed with other metals, the metals to be alloyed with the magnesium are introduced in a liquid condition into the phase of condensation of the magnesium.

15. A process for obtaining very pure magnesium, which comprises mixing intimately a bath of molten magnesium fluoride with a reducing agent of the group consisting of calcium and the metalloids of the group consisting of carbon and silicon, heating the mixture at the temperature of distillation of the magnesium and in a non-oxidizing atmosphere, condensing the magnesium vapors which are formed, as they are evolved, on a pure magnesium bath in a molten condition, treating the fluorinated slag which forms the residue of the reaction, as it is formed, to form therefrom hydrofluoric acid, causing said hydrofluoric acid to act on a magnesium ore in order to form magnesium fluoride and introducing said magnesium fluoride into the bath of molten magnesium fluoride in course of reduction.

16. A cyclic process for obtaining very pure magnesium according to claim 15, in which, in order to obtain magnesium alloyed with other metals, stable and reducible fluorides of the metals to be alloyed with the magnesium are mixed with the bath of molten magnesium fluoride, the hydrofluoric acid formed from the slag which forms the residue of the reduction reaction being caused to act on a mixture of magnesium ore and of ores of the metals to be alloyed with the magnesium.

17. A cyclic process for obtaining very pure magnesium, which comprises treating magnesiferous ore with hydrofluoric acid to form magnesium fluoride, treating said magnesium fluoride with calcium in the state of a compound with a metalloid of the group consisting of carbon and silicon at the temperature of distillation of the magnesium and in a non-oxidizing atmosphere, condensing the magnesium vapors resulting from the reducing treatment, treating the fluorinated product remaining after the distillation of the magnesium to regenerate the hydrofluoric

acid, treating a further quantity of magnesiferous ore with said hydrofluoric acid to form magnesium fluoride, and treating said magnesium fluoride with calcium in the state of a compound with a metalloid of the group consisting of carbon and silicon at the temperature of the distillation of the magnesium and in a non-oxidizing atmosphere.

18. A cyclic process for obtaining very pure magnesium according to claim 17, in which calcium in the state of calcium carbide is used for the reduction of the magnesium fluoride.

19. A cyclic process for obtaining very pure magnesium, which comprises treating magnesiferous ore with hydrofluoric acid to form magnesium fluoride, treating said magnesium fluoride with a metalloid of the group consisting of carbon and silicon in the state of an alloy with a non-reducing metal at the temperature of distillation of the magnesium and in a non-oxidizing atmosphere, condensing the magnesium vapors resulting from the reducing treatment, treating the fluorinated product remaining after the distillation of the magnesium to regenerate the hydrofluoric acid, treating a further quantity of magnesiferous ore with said hydrofluoric acid to form magnesium fluoride, and treating said magnesium fluoride with a metalloid of the group consisting of carbon and silicon in the state of an alloy with a non-reducing metal at the temperature of the distillation of the magnesium and in a non-oxidizing atmosphere.

20. A cyclic process for obtaining very pure magnesium according to claim 19, in which silicon in the state of a ferro-silicon alloy having a high content of silicon is used for the reduction of the magnesium fluoride.

21. A cyclic process for obtaining very pure magnesium, which comprises treating magnesiferous ore with hydrofluoric acid to form magnesium fluoride, treating said magnesium fluoride with a metalloid of the group consisting of carbon and silicon in the state of an alloy with several metals at the temperature of distillation of the magnesium and in a non-oxidizing atmosphere, condensing the magnesium vapors resulting from the reducing treatment, treating the fluorinated product remaining after the distillation of the magnesium to regenerate the hydrofluoric acid, treating a further quantity of magnesiferous ore with said hydrofluoric acid to form magnesium fluoride, and treating said magnesium fluoride with a metalloid of the group consisting of carbon and silicon in the state of an alloy with several metals at the temperature of the distillation of the magnesium and in a non-oxidizing atmosphere.

22. A cyclic process for obtaining very pure magnesium according to claim 21, in which silicon in the state of an alloy of silicon, iron and aluminum having a high content of silicon and aluminum is used for the reduction of the magnesium fluoride.

23. A cyclic process for obtaining very pure magnesium according to claim 21, in which silicon in the state of an alloy of silicon, iron and aluminum containing about 50% of silicon, 15% of iron and 35% of aluminum is used for the reduction of the magnesium fluoride, in such a proportion that finally an alloy of iron and silicon containing 60% of iron and 40% of silicon is obtained.

CARLO ADAMOLI.